

April 28, 1970

V. K. CHANDHOK ET AL

3,508,912

TOOL STEEL CONTAINING CHROMIUM AND COBALT

Filed May 26, 1969

5 Sheets-Sheet 1

FIG. 1



FIG. 2



INVENTORS.

VIJAY K. CHANDHOK and  
AUGUST KASAK

By

*John A. Pagan*  
Attorney

April 28, 1970

V. K. CHANDHOK ET AL

3,508,912

TOOL STEEL CONTAINING CHROMIUM AND COBALT

Filed May 26, 1969

5 Sheets-Sheet 2

FIG. 3.



FIG. 4.



INVENTORS.  
VIJAY K. CHANDHOK and  
AUGUST KASAK

By

*John R. Regan*  
Attorney

April 28, 1970

V. K. CHANDHOK ET AL

3,508,912

TOOL STEEL CONTAINING CHROMIUM AND COBALT

Filed May 26, 1969

5 Sheets-Sheet 3

FIG. 5



FIG. 7



INVENTORS.  
VIJAY K. CHANDHOK and  
AUGUST KASAK

By

*John A. Pagan*  
Attorney

April 28, 1970

V. K. CHANDHOK ET AL.

3,508,912

TOOL STEEL CONTAINING CHROMIUM AND COBALT

Filed May 26, 1969

5 Sheets-Sheet 4

FIG. 6



FIG. 10



INVENTORS.  
VIJAY K. CHANDHOK and  
AUGUST KASAK

John R. Pegan  
Attorney

April 28, 1970

V. K. CHANDHOK ET AL

3,508,912

TOOL STEEL CONTAINING CHROMIUM AND COBALT

Filed May 26, 1969

5 Sheets-Sheet 5



INVENTORS.  
VIJAY K. CHANDHOK and  
AUGUST KASAK  
By

*John R. Pagan*  
Attorney

**3,508,912**  
**TOOL STEEL CONTAINING CHROMIUM**  
**AND COBALT**

Vijay K. Chandhok, Mount Lebanon, and August Kasak, Upper St. Clair, Pa., assignors to Crucible Inc., Pittsburgh, Pa., a corporation of Delaware  
 Continuation-in-part of application Ser. No. 514,076, Dec. 15, 1965. This application May 26, 1969, Ser. No. 830,920

Int. Cl. C22c 39/20

U.S. Cl. 75—128

2 Claims 10

**ABSTRACT OF THE DISCLOSURE**

This invention relates to a tool steel that may be machined in the austenitized and quenched condition and then age-hardened. The composition, in percent, is carbon+nitrogen up to .08, chromium 2.5 to 6, molybdenum 3 to 12, cobalt 8 to 15, nickel up to 4, cobalt+nickel 10 to 18, manganese up to 1, balance iron.

This application is a continuation-in-part of our co-pending application Ser. No. 514,076, filed Dec. 15, 1965.

Traditionally, tool steels of the prior art, hot work steels as well as cutting tool steels, depends, by and large, upon the presence in the steel microstructure of simple or complex carbides to provide the necessary strength and wear resistance.

However, the presence of substantial amounts of carbon in the alloy, and the consequent presence of microstructural carbides, in the useful condition of heat treatment of the steel, causes serious difficulties in the processing and use of conventional prior art tool steels. Thus, carbon and carbides tend to become severely segregated during the solidification of ingots, and this segregation leads to inhomogeneities in the tool steel products made from such ingots, even after large amounts of working. The result is inconsistent tool performance and more or less severe embrittlement and consequent breakage in use. Moreover, carbon-containing tool steels are subject to loss of carbon under the decarburizing environmental conditions often encountered during mill processing, heat treatment, and tool manufacture and service use. As is well known, decarburization detracts considerably from the usefulness of the steel in tool steel applications and may, indeed, necessitate the use of other, more expensive and otherwise less satisfactory alloys in many instances.

A further property requirement in many, if not most, tool steel applications is that the product must be shaped or finished by machining to a final desired configuration, so that machinability of the steel is important. The carbon-containing tool steels must be machined in an annealed condition due to the hardness and relative brittleness of the ferrite-carbide structure that exists at low temperatures. Following machining, a full heat treatment, consisting of austenitizing, quenching or air cooling, and tempering, is necessary to attain the optimum combination of properties for service.

The austenitizing heat treatment, as aforesaid, necessitates the use of high temperatures, e.g., about 1800° F. to 2400° F., and, as a consequence of the dimensional changes attendant upon phase transformations during such heat treatment, warpage of a finished machined tool or tool part is a frequent occurrence. This is particularly troublesome in the case of articles of complex configurations. Additionally, the required high austenitizing temperatures are productive of appreciable surface scaling and/or decarburization unless the environmental conditions are carefully controlled. Such protective procedures are, of course, time consuming and costly. Post-austenitizing corrective finishing operations are often required.

As a rule, articles fabricated from the carbon-containing, hardenable tool steels of the prior art must be tempered immediately following the austenitizing heat treatment because strain cracking of the article is otherwise likely. The medium- or high-carbon martensite resulting from the austenitizing treatment is very brittle so that cracks are prone to occur due to severe internal stresses created by non-uniform cooling rates across the article cross section, or as a result of different cooling rates of cross-sectional variations in complex article shapes.

Carbon-containing hot work tool steels of the prior art all suffer from heat checking to a greater or lesser degree. Such steels in service are exposed to relatively high surface temperatures, while a short distance beneath the surface, the temperature is much lower. Such conditions are productive of tremendous fatigue stresses which, upon repeated cycling, cause the formation of small surface cracks which, growing in size and extent, constitute the familiar heat checking condition.

Accordingly, it is an object of the present invention to provide new and improved tool steels which are substantially free of the disadvantages of prior art tool steels containing substantial amounts of carbon.

It is another object of this invention to provide tool steels which are heat hardenable by means other than carbide formation, specifically steels which are hardenable by the precipitation in the steel microstructure of intermetallic compounds, as compounds of the elements iron, molybdenum, tungsten and chromium.

It is still another object of the invention to provide new and improved steels which are readily machinable in an austenitized condition and thereafter hardenable at a relatively lower temperature to avoid high temperature dimensional changes and surface deterioration.

It is yet another object to provide new and improved hot work die steels which exhibit the aforesaid objectives and which have an enhanced resistance to heat checking.

It is a further object to provide new and improved, substantially carbon-free cutting tool steels which are hardenable by intermetallic compound precipitation upon tempering.

In accordance with the foregoing objects, the invention constitutes a hot work steel consisting essentially of, by weight percent, carbon+nitrogen up to .08 chromium 2.5 to 6, molybdenum 3 to 10 or 12, cobalt 8 to 15, nickel up to 4, cobalt+nickel 10 to 18, manganese up to 1 and balance iron.

The foregoing and other objects of the invention will be more readily apparent from the following description and drawings wherein:

FIGURE 1 comprises a series of graphs constituting tempering curves, at various austenitizing temperatures from 1700 to 2200° F., showing the change in hardness with change in tempering temperature between 1000° F. and 1350° F., for an inventive steel particularly suited for use as a hot work die steel;

FIGURE 2 comprises a series of tempering curves similar to those of FIG. 1, for a steel of the invention particularly suitable for use as a cutting tool steel;

FIGURE 3 comprises a series of graphs relating the chromium content of experimental steels with the room temperature and elevated temperature strength properties of the steels;

FIGURE 4 is illustrative of, first, the relationship between molybdenum content of certain experimental steels and the maximum attainable tempered hardness thereof, and, second, the effect of that element upon the tempering resistance of those steels, expressed in terms of the percentage difference between the maximum hardness and the hardness observed at progressively higher tempering temperatures;

FIGURE 5 constitutes a series of graphs relating the room temperature and elevated temperature strength properties to the proportion of tungsten in the total content of molybdenum plus one-half the tungsten in an approximately 0.05C-5Cr-7.5 (Mo+½W)-13(Co+Ni) base composition;

FIGURE 6 constitutes a pair of graphs comparing the tempering resistance of a high hardness steel of the invention (useful as a cutting tool steel) and that of a currently commonly used high speed steel;

FIGURE 7 comprises a series of graphs relating the cobalt content of experimental steels with the room temperature and elevated temperature strength properties of the steels;

FIGURE 8 constitutes a series of graphs relating the cobalt content of experimental steels with the spread in hardness in the austenitized condition and in a hardened condition after tempering;

FIGURE 9 constitutes a series of graphs relating the room temperature and elevated temperature strength properties to the proportion of nickel in the total content of cobalt plus nickel in an approximately 0.05C-5Cr-7.7 Mo-13.5 to 15(Co+Ni) base composition, and

FIGURE 10 constitutes a series of graphs illustrative of the comparative temper resistance of a representative inventive steel with that of prior art hot work and heat resistant stainless steels.

In contrast to conventional tool steels of the prior art, the steels of the invention are carbon-free, or contain only residual amounts of carbon introduced into the steel incidentally to conventional steelmaking practices. The inventive steels derive their strength and wear resistance principally from the precipitation of intermetallic compounds upon aging (tempering) at elevated temperatures. By a proper proportioning of the several essential alloying elements, and by the use of a proper heat treatment, the new steels can be hardened to high hardnesses, as 60-65 Rockwell C, i.e., in the high speed steel hardness range.

do not exist, and, consequently, no special measures are needed to prevent this undesirable occurrence during mill processing, heat treatment, article manufacture, or in-service application.

A further important advantage of our new steels is that no high temperature (e.g., 1400-2400° F.) heat treatment is required after machining of the steels in the austenitized condition. Only a relatively low temperature aging or tempering treatment, e.g., at about 1000-1100° F., is needed after finish machining to impart to the optimum tool steel properties. Consequently, previously necessary steps in the tool manufacturing operation can be eliminated and, quite importantly, difficulties arising from dimensional distortion and scaling during final heat treatment are avoided or minimized.

The martensite formed in those low-carbon or substantially carbon-free steels is considerably softer and tougher than that formed in hardenable medium- or high-carbon tool steels. Consequently, these new steels retain relatively low hardness values and are readily amenable to easy machining prior to subsequent age hardening to much higher, final hardnesses. Moreover, the new steels avoid or minimize the tendency toward strain cracking on cooling.

When compositionally controlled as taught herein, the steels of the invention are producible free and substantially free of free ferrite, and accordingly exhibit a high degree of dimensional stability and hot workability.

A first series of experimental steels was prepared by levitation melting in the form of 15 gram button ingots, and the small ingots were then processed to sheet form, heat treated (austenitized, quenched, refrigerated and then aged), and then tested for hardness. The compositions of these steels, the heat treatment conditions, and the hardness values so obtained, are given in Table I. In each case, austenitization was carried out at 2100° F. for one half hour. Refrigeration of each of the test specimens was done at -100° F. for one half hour.

TABLE I

| Steel No.: | Composition, weight percent |      |      |      |     |            | After austenitization at 2,100° F. for ½ hour; oil quenched | After refrigeration at -100° F. for ½ hour | Tempered 2+2 hours at indicated temperature, then air cooled |           |           |           |
|------------|-----------------------------|------|------|------|-----|------------|-------------------------------------------------------------|--------------------------------------------|--------------------------------------------------------------|-----------|-----------|-----------|
|            | C                           | Cr   | Mo   | Co   | V   | Fe         |                                                             |                                            | 900° F.                                                      | 1,000° F. | 1,100° F. | 1,200° F. |
| 1.....     | 0.10                        | 14.0 | 10.0 | 13.5 | 0.5 | Balance... | 31.0                                                        | 33.5                                       | 44.5                                                         | 47.5      | 56.0      | 54.0      |
| 1A.....    | 0.10                        | 14.0 | 10.0 | 13.5 | 0.5 | do         | 31.0                                                        | 35.0                                       | 42.5                                                         | 52.0      | 55.0      | 60.0      |
| 2.....     | 0.10                        | 14.0 | 15.0 | 13.5 | 0.5 | do         | 44.0                                                        | 42.5                                       | 45.5                                                         | 51.0      | 60.0      | 60.0      |
| 2A.....    | 0.10                        | 14.0 | 15.0 | 13.5 | 0.5 | do         | 44.5                                                        | 45.5                                       | 42.0                                                         | 48.0      | 56.0      | 53.5      |
| 3.....     | 0.10                        | 7.0  | 8.0  | 13.5 | 0.5 | do         | 41.5                                                        | 41.0                                       | 41.0                                                         | 49.0      | 55.0      | 57.0      |
| 3A.....    | 0.10                        | 7.0  | 8.0  | 13.5 | 0.5 | do         | 41.0                                                        | 41.0                                       | 40.5                                                         | 40.5      | 60.0      | 57.0      |
| 4.....     | 0.10                        | 7.0  | 10.0 | 13.5 | 0.5 | do         | 40.5                                                        | 41.0                                       | 40.0                                                         | 49.0      | 55.0      | 57.0      |
| 4A.....    | 0.10                        | 7.0  | 10.0 | 13.5 | 0.5 | do         | 40.0                                                        | 40.5                                       | 40.0                                                         | 47.5      | 53.0      | 59.0      |
| 5.....     | 0.10                        | 5.0  | 10.0 | 13.5 | 0.5 | do         | 40.0                                                        | 40.5                                       | 38.0                                                         | 38.5      | 59.0      | 56.5      |
| 5A.....    | 0.10                        | 5.0  | 10.0 | 13.5 | 0.5 | do         | 40.0                                                        | 40.5                                       | 38.0                                                         | 38.5      | 59.0      | 56.5      |

Moreover, the steels of this invention are extremely temper resistant, retaining strengths and hardnesses, at temperatures of 1100 to 1400° F. or higher, clearly superior to other, known commercial tool steels.

Additionally, since the steels of the invention do not depend on carbon for production of the necessary property characteristics, the problems usually arising as a result of decarburization of carbon-containing tool steels

The Table I data is illustrative of the unexpectedly high hardness values obtained on tempering these essentially carbon-free steels at temperatures up to 1200° F.

A further series of steels was prepared as 10-pound, induction melted heats, these heats processed to bar form, and similarly heat treated and tested for aging hardness response and tempering resistance. The compositions of this second series of steels is given in Table II.

TABLE II

| Steel No.: | Bar No. | Composition, weight percent |       |      |       |       |       |      |      |       |          |
|------------|---------|-----------------------------|-------|------|-------|-------|-------|------|------|-------|----------|
|            |         | C                           | N     | Cr   | Mo    | Co    | Ni    | Mn   | Si   | S     | Fe       |
| HW1.....   | 62-237  | 0.107                       | ..... | 5.12 | 10.01 | 13.84 | ..... | 0.22 | 0.12 | 0.009 | Balance. |
| HW2.....   | 62-238  | 0.006                       | ..... | 6.89 | 9.95  | 14.08 | ..... | 0.20 | 0.16 | 0.008 | Do.      |
| HW3.....   | 62-239  | 0.105                       | ..... | 5.05 | 8.91  | 14.12 | ..... | 0.22 | 0.15 | 0.009 | Do.      |
| HW4.....   | 62-240  | 0.102                       | ..... | 5.12 | 11.90 | 13.84 | ..... | 0.36 | 0.24 | 0.010 | Do.      |
| HW5.....   | 62-241  | 0.103                       | ..... | 9.72 | 15.00 | 13.84 | ..... | 0.48 | 0.30 | 0.008 | Do.      |
| HW6.....   | 62-339  | 0.110                       | 0.02  | 5.03 | 9.04  | 12.09 | 2.25  | 0.16 | 0.13 | 0.009 | Do.      |
| HW7.....   | 62-340  | 0.106                       | 0.02  | 4.99 | 9.04  | 13.85 | 0.09  | 0.19 | 0.14 | 0.009 | Do.      |
| HW8.....   | 62-344  | 0.108                       | 0.01  | 5.10 | 9.30  | 13.92 | 0.09  | 0.18 | 0.11 | 0.009 | Do.      |
| HW9.....   | 63-5    | 0.016                       | ..... | 6.45 | 9.41  | 9.86  | 4.26  | 0.16 | 0.12 | 0.012 | Do.      |
| HW10.....  | 63-125  | 0.028                       | 0.005 | 3.59 | 7.35  | 10.96 | 2.08  | 0.10 | 0.11 | 0.015 | Do.      |

The test conditions to which the Table II steels were subjected, and the results thereof, are set forth in Table III.

steels, as HW1, HW2, HW3, HW6-HW9, are hardenable to about 57-61 R<sub>c</sub> on tempering at 1100° F. after austenitizing at 2200° F. Substantial and highly useful hard-

TABLE III  
[Results of Tempering Studies on the Table II Steels<sup>1</sup>]

| Steel                             | Austen-<br>itizing<br>temper-<br>ature,<br>° F. |       | As<br>rolled |      | As<br>quenched<br>plus<br>refrig-<br>erated |      | Hardness (R <sub>c</sub> ) |           |           |                  |           |           |
|-----------------------------------|-------------------------------------------------|-------|--------------|------|---------------------------------------------|------|----------------------------|-----------|-----------|------------------|-----------|-----------|
|                                   |                                                 |       |              |      |                                             |      | Tempered                   |           |           | Cumulatively at— |           |           |
|                                   |                                                 |       |              |      |                                             |      | 1,000° F.                  | 1,100° F. | 1,200° F. | 1,300° F.        | 1,350° F. | 1,400° F. |
| HW1, 0.10 C-6 Cr-10 Mo-14 Co      | 2,200                                           | ----- | 42           | 44.5 | 46                                          | 62   | 61                         | 56        | 47        | 44               | -----     | -----     |
|                                   | 2,100                                           | ----- | 43.5         | 46   | 59.5                                        | 61.5 | 61                         | 55.5      | 46.5      | 40.5             | -----     | -----     |
|                                   | 2,000                                           | ----- | 41           | 44.5 | 41                                          | 59.5 | 59.5                       | 54        | 45.5      | 39.5             | -----     | -----     |
|                                   | 1,900                                           | ----- | 39.5         | 40   | 55.5                                        | 57.5 | 52                         | 44        | 38        | -----            | -----     | -----     |
|                                   | 1,800                                           | ----- | 40           | 40   | 53.5                                        | 55.5 | 49.5                       | 42        | 37        | -----            | -----     | -----     |
|                                   | 1,700                                           | 45.5  | 39           | 39   | 50                                          | 51.5 | 45.5                       | 39        | 36.5      | 31               | -----     | -----     |
| HW2, 0.10 C-7 Cr-10 Mo-14 Co      | 2,200                                           | ----- | 45           | 46.5 | 62.5                                        | 60.5 | 56.5                       | 49        | 44        | -----            | -----     | -----     |
|                                   | 2,100                                           | ----- | 44.5         | 46.5 | 63.5                                        | 61.5 | 56.5                       | 49        | 39        | -----            | -----     | -----     |
|                                   | 2,000                                           | ----- | 42           | 44   | 61.5                                        | 60   | 54.5                       | 46.5      | 40        | -----            | -----     | -----     |
|                                   | 1,900                                           | ----- | 42           | 43   | 58                                          | 58   | 53                         | 45.5      | 41.5      | -----            | -----     | -----     |
|                                   | 1,800                                           | ----- | 41           | 41.5 | 55.5                                        | 56   | 50.5                       | 43.5      | 38.5      | -----            | -----     | -----     |
|                                   | 1,700                                           | 47    | 41           | 40   | 51                                          | 52   | 47.5                       | 41.5      | 39.5      | 37.5             | -----     | -----     |
| HW3, 0.10 C-5Cr-9 Mo-14 Co        | 2,200                                           | ----- | 47           | 48   | 60.5                                        | 60   | 55                         | 45.5      | 40        | -----            | -----     | -----     |
|                                   | 2,100                                           | ----- | 44.5         | 45.6 | 58                                          | 59.5 | 53.5                       | 42        | 37        | -----            | -----     | -----     |
|                                   | 2,000                                           | ----- | 43.5         | 44.5 | 58                                          | 58   | 52                         | 43        | 37        | -----            | -----     | -----     |
|                                   | 1,900                                           | ----- | 42           | 42.5 | 55.5                                        | 56   | 51                         | 43        | 34.5      | -----            | -----     | -----     |
|                                   | 1,800                                           | ----- | 40           | 40.5 | 53                                          | 55   | 50.5                       | 43        | 36.5      | -----            | -----     | -----     |
|                                   | 1,700                                           | 46    | 39.5         | 38.5 | 49                                          | 51.5 | 46.5                       | 40        | 35.5      | 34               | -----     | -----     |
| HW4, 0.10 C-5 Cr-12 Mo-14 Co      | 2,200                                           | ----- | 40           | 42.5 | 64.5                                        | 63   | 58.5                       | 51.5      | 45.5      | -----            | -----     | -----     |
|                                   | 2,100                                           | ----- | 42           | 44.5 | 63.5                                        | 62   | 57.5                       | 50        | 43.5      | -----            | -----     | -----     |
|                                   | 2,000                                           | ----- | 42           | 44   | 61.5                                        | 60.5 | 56                         | 47.5      | 42        | -----            | -----     | -----     |
|                                   | 1,900                                           | ----- | 43           | 43.5 | 58.5                                        | 58.5 | 53.5                       | 44        | 39        | -----            | -----     | -----     |
|                                   | 1,800                                           | ----- | 42.5         | 43   | 55                                          | 56.5 | 49                         | 42        | 38.5      | -----            | -----     | -----     |
|                                   | 1,700                                           | 44    | 48.5         | 42   | 51.5                                        | 53.5 | 45                         | 41.5      | 40        | 38.5             | -----     | -----     |
| HW5, 0.10 C-10 Cr-15 Mo-14 Co     | 2,200                                           | ----- | 50           | 50   | 62.5                                        | 64   | 62                         | 57        | 53        | -----            | -----     | -----     |
|                                   | 2,100                                           | ----- | 41           | 41.5 | 62                                          | 63   | 60.5                       | 56        | 51.5      | -----            | -----     | -----     |
|                                   | 2,000                                           | ----- | 49.5         | 49.5 | 64                                          | 62.5 | 59.5                       | 55        | 50        | -----            | -----     | -----     |
|                                   | 1,900                                           | ----- | 49.5         | 50   | 61.5                                        | 61   | 57.5                       | 52.5      | 50        | -----            | -----     | -----     |
|                                   | 1,800                                           | ----- | 49           | 49.5 | 59.5                                        | 59.5 | 56.5                       | 51.5      | 50.5      | 50.5             | 50.5      | 50.5      |
| HW6, 0.10 C-5 Cr-9 Mo-12 Co-2 Ni  | 2,200                                           | 44    | 43           | 43.5 | 61.5                                        | 59   | 54                         | 44        | 39.5      | 35               | -----     | -----     |
|                                   | 2,100                                           | 44    | 42           | 42.5 | 62                                          | 59   | 54                         | 44.5      | 39        | 34.5             | -----     | -----     |
|                                   | 2,000                                           | 45    | 40.5         | 41   | 60                                          | 57.5 | 51                         | 42        | 36.5      | 33.5             | -----     | -----     |
|                                   | 1,900                                           | 46.0  | 39           | 40   | 57                                          | 55.5 | 49                         | 40        | 36        | 33.5             | -----     | -----     |
|                                   | 1,800                                           | 44.5  | 33.5         | 34   | 55                                          | 55   | 49                         | 40.5      | 35.5      | 33.5             | -----     | -----     |
|                                   | 1,700                                           | 48    | 36.5         | 37.5 | 52.5                                        | 52.5 | 46.5                       | 38.5      | 35        | 33               | -----     | -----     |
| HW7, 0.10 C-5 Cr-9 Mo-14 Co       | 2,200                                           | 44    | 40           | 41   | 59.5                                        | 60   | 55.5                       | 44.5      | 40        | 35.5             | -----     | -----     |
|                                   | 2,100                                           | 45.5  | 40           | 41.5 | 58.5                                        | 60   | 55.5                       | 46        | 40.5      | 35               | -----     | -----     |
|                                   | 2,000                                           | 46    | 40.5         | 41.5 | 56                                          | 59.5 | 53.5                       | 44.5      | 39        | 33.5             | -----     | -----     |
|                                   | 1,900                                           | 46.5  | 39           | 39.5 | 53.5                                        | 57   | 51.5                       | 41.5      | 37.5      | 33.5             | -----     | -----     |
|                                   | 1,800                                           | 46.5  | 38           | 38.5 | 51                                          | 55   | 50                         | 41        | 36        | 32               | -----     | -----     |
| HW8, 0.02 C-6 Cr-9 Mo-10 Co-4 Ni  | 2,200                                           | ----- | 36           | 35   | 59                                          | 57   | 52.5                       | 48        | 45        | 43               | -----     | -----     |
|                                   | 2,100                                           | ----- | 35.5         | 35   | 60                                          | 57.5 | 52                         | 48        | 45        | 43               | -----     | -----     |
|                                   | 2,000                                           | ----- | 35.5         | 35   | 59.5                                        | 57   | 52.5                       | 47.5      | 44        | 42               | -----     | -----     |
|                                   | 1,900                                           | ----- | 37           | 36.5 | 58                                          | 55   | 50.5                       | 45.5      | 41        | 39.5             | -----     | -----     |
|                                   | 1,800                                           | ----- | 40.5         | 39.5 | 56.5                                        | 53.5 | 49                         | 42.5      | 39.5      | 40.5             | -----     | -----     |
|                                   | 1,700                                           | ----- | 41.5         | 40.5 | 55                                          | 52.5 | 47.5                       | 42.5      | 41.5      | 41.5             | -----     | -----     |
|                                   | 1,600                                           | ----- | 43           | 42   | 53                                          | 51   | 46.5                       | 43.5      | 42.5      | 42.5             | 42        | 42        |
|                                   | 1,500                                           | ----- | 44.5         | 44   | 51.5                                        | 50   | 46.5                       | 44.5      | 43.5      | 42.5             | 42.5      | 42.5      |
| HW10, 0.03 C-5 Cr-7 Mo-11 Co-2 Ni | 2,200                                           | 41.5  | 34           | 34   | 52                                          | 53.5 | 48.5                       | 44.5      | 40.5      | 36               | -----     | -----     |
|                                   | 2,100                                           | 39    | 34.5         | 34   | 52.5                                        | 53.5 | 49                         | 44.5      | 40.5      | 35.5             | -----     | -----     |
|                                   | 2,000                                           | 40    | 34.5         | 34   | 53                                          | 53.5 | 49                         | 44.5      | 40.5      | 36               | -----     | -----     |
|                                   | 1,900                                           | 40.5  | 36           | 36   | 53.5                                        | 54   | 49.5                       | 44.5      | 40        | 36               | -----     | -----     |
|                                   | 1,800                                           | 41.5  | 36.5         | 36   | 53                                          | 53.5 | 48.5                       | 41.5      | 36.5      | 33               | -----     | -----     |
|                                   | 1,700                                           | 40    | 38.5         | 37.5 | 51                                          | 51   | 45.5                       | 38.5      | 36        | 34.5             | -----     | -----     |
|                                   | 1,600                                           | 40    | 37.5         | 37   | 48.5                                        | 48.5 | 44                         | 39        | 37        | 36               | -----     | -----     |
|                                   | 1,500                                           | 39    | 38           | 37   | 44.5                                        | 45   | 42                         | 39        | 38        | 36.5             | -----     | -----     |

<sup>1</sup> Specimens austenitized at the indicated temperature, oil quenched, refrigerated at -100° F. for 1/2 hour, and cumulatively tempered at successively higher indicated temperatures for 2+2 hours.

It will be seen from the Table III test results that the experimental steels there studied are hardenable from relatively low quenched (or quenched and refrigerated) hardnesses on the order of 37-40 R<sub>c</sub> (1700° F. austenitizing temperature) or 34-50 R<sub>c</sub> (2200° F. austenitizing temperature) to much higher tempered or aged hardness levels. For example, the lower (7-10%) molybdenum

70 hardnesses, e.g., about 40-45 R<sub>c</sub>, are retained to tempering temperatures as high as 1350° F., thereby showing the extreme temper resistance and useful high temperature applicability of these steels. These advantageous properties are graphically illustrated in FIG. 1, where the Table II data for Steel HW3 are plotted as a series of 75 tempering curves showing the change in hardness of

that steel with tempering temperatures between 1000° F. and 1350° or 1400° F. for each of the Table II austenitization temperatures from 1700° to 2200° F. As will be seen from FIG. 1, peak hardness occurs, in each instance, at a tempering temperature of about 1000–1100° F., and maximum hardness, about 60 R<sub>c</sub>, is obtained at the highest austenitizing temperature, 2200° F. Such steels find particular application as hot work steels.

Similarly, the higher (12–15%) molybdenum steels, HW4 and HW5, are hardenable from quenched hardnesses of about 43–50 R<sub>c</sub>, after a 2200° F. austenitizing treatment, to very high aged hardnesses of about 63–65 R<sub>c</sub>. In these steels, hardnesses of about 46–53 R<sub>c</sub> are retained after tempering at temperatures as high as 1350° F. Illustratively, the Table II data for Steel HW4 is graphically shown in FIG. 2, wherein the similarity to the FIG. 1 steels is seen together with the higher peak hardnesses which particularly suit these steels for cutting applications.

A third series of steels was also prepared, as 10-pound heats, processed to bar form, and subjected to extensive investigation of hardness, room temperature and elevated temperature strength properties, impact strength, and ductility. The compositions of these latter steels are given in Table IV.

Characteristically, the inventive steels are essentially carbon-free, but it is realized that a certain carbon content is necessary to make the steels satisfactorily producible by conventional steelmaking practices. Test results show that an increase in carbon above 0.08% (Steels HW12, 13, and 15, Table V) resulted in a gradual drop in both the room-temperature and elevated-temperature strength properties. Hence, carbon or carbon+nitrogen may be present in amounts up to 0.08%.

Since the steel is intended for use at elevated temperatures in an essentially air atmosphere, some chromium is desirable to provide satisfactory oxidation (scaling) resistance. Also, test results show that the tempering resistance is somewhat increased by 2.5 or 6% chromium (HW17 and 12 vs. HW14, Table V). At the 11.1% level (HW19, Table V), 20% delta (free) ferrite formed in the microstructure upon austenitizing at 1800° F. and the room-temperature and elevated-temperature strength properties and ductility (elongation, reduction of area, and impact value) declined. Hence, chromium is present within in the range of 2.5 to 6%.

Molybdenum is an important strengthening agent in the steel. The tempering resistance is steadily increased with increasing molybdenum content, but the ductility is lowered. At 10% molybdenum (HW21, Table V), some free (delta) ferrite is formed upon austenitizing at 1800° F.

TABLE IV

| Heat No.          | Bar No. | Composition, weight percent |       |       |       |       |       |       |       |       |      |       |          |
|-------------------|---------|-----------------------------|-------|-------|-------|-------|-------|-------|-------|-------|------|-------|----------|
|                   |         | C                           | N     | Cr    | W     | Mo    | Co    | Ni    | Mn    | Si    | S    | Fe    |          |
| <b>Steel No.:</b> |         |                             |       |       |       |       |       |       |       |       |      |       |          |
| HW12              | 1140    | 63-309                      | 0.036 | 0.01  | 5.19  | ----- | 7.70  | 11.16 | 2.15  | ----- | 0.03 | 0.013 | Balance. |
| HW13              | 1141    | 63-310                      | 0.095 | 0.01  | 5.15  | ----- | 7.37  | 11.22 | 2.15  | ----- | 0.05 | 0.012 | Do.      |
| HW15              | 1142    | 63-311                      | 0.049 | 0.01  | 0.40  | ----- | 7.30  | 10.93 | 2.18  | ----- | 0.03 | 0.012 | Do.      |
| HW14              | 1143    | 63-312                      | 0.161 | 0.01  | 5.33  | ----- | 7.63  | 11.10 | 2.14  | ----- | 0.05 | 0.012 | Do.      |
| HW16              | 1144    | 63-313                      | 0.051 | 0.01  | 2.68  | ----- | 7.60  | 10.88 | 2.05  | ----- | 0.05 | 0.013 | Do.      |
| HW17              | 1145    | 63-314                      | 0.063 | 0.01  | 2.85  | ----- | 8.29  | 10.93 | 2.28  | ----- | 0.07 | 0.012 | Do.      |
| HW18              | 1146    | 63-315                      | 0.037 | 0.02  | 5.78  | ----- | 3.64  | 11.00 | 2.14  | ----- | 0.06 | 0.009 | Do.      |
| HW19              | 1147    | 63-316                      | 0.052 | 0.03  | 11.14 | ----- | 7.70  | 11.41 | 2.20  | ----- | 0.12 | 0.009 | Do.      |
| HW20              | 1148    | 63-317                      | 0.047 | 0.02  | 5.46  | ----- | 9.95  | 11.41 | 2.15  | ----- | 0.15 | 0.011 | Do.      |
| HW21              | 1149    | 63-318                      | 0.049 | 0.02  | 5.17  | ----- | 15.13 | 11.07 | 2.15  | ----- | 0.13 | 0.014 | Do.      |
| HW22              | 1150    | 62-319                      | 0.036 | 0.02  | 5.30  | ----- | 7.57  | 8.00  | 2.14  | ----- | 0.08 | 0.010 | Do.      |
| HW23              | 1151    | 63-320                      | 0.046 | 0.02  | 5.37  | ----- | 7.51  | 8.07  | ----- | ----- | 0.06 | 0.010 | Do.      |
| HW24              | 1152    | 63-321                      | 0.051 | 0.02  | 5.39  | ----- | 7.37  | 11.15 | ----- | ----- | 0.08 | 0.011 | Do.      |
| HW25              | 1153    | 63-322                      | 0.053 | 0.02  | 5.42  | ----- | 7.63  | 14.88 | ----- | ----- | 0.16 | 0.011 | Do.      |
| HW26              | 1154    | 63-323                      | 0.043 | 0.01  | 5.53  | ----- | 7.63  | 9.22  | 4.01  | ----- | 0.14 | 0.010 | Do.      |
| HW27              | 1155    | 63-324                      | 0.042 | 0.01  | 5.32  | ----- | 7.76  | 6.88  | 6.58  | ----- | 0.07 | 0.011 | Do.      |
| HW29              | 1156    | 63-325                      | 0.047 | 0.02  | 5.27  | 7.30  | 3.90  | 11.38 | 2.16  | ----- | 0.07 | 0.011 | Do.      |
| HW30              | 1157    | 63-326                      | 0.046 | 0.01  | 5.11  | 14.55 | ----- | 11.41 | 2.1   | 0.02  | 0.02 | 0.009 | Do.      |
| HW41              | 1267    | 64-46                       | 0.080 | ----- | 5.31  | ----- | 7.49  | 17.66 | ----- | 0.20  | 0.06 | ----- | Do.      |

Table V sets forth the nominal compositions of the Table IV steels, rearranged in groups having an approximately constant base composition and wherein one or a pair of elements is varied in amount or proportion (such variable elements being italicized in Table V). The test conditions and observed property characteristics are also shown in Table V, Column 9.

Many of the standard tensile test specimens of the Table IV steels were prepared by machining in the as-austenitized condition. Machine fixtures and dies have also been similarly produced from the inventive steels.

The foregoing experimental data, especially that of Table V, shows that the steels of this invention possess high aged hardness, a considerable spread between quenched and aged hardness (thus permitting machining in the autenitized condition and subsequent age hardening), high resistance to softening upon exposure to elevated temperatures, high strength over a wide temperature range, and reasonably good ductility—all desirable characteristics of superior materials for hot work tool and high-performance cutting tool applications.

Above 10% (HW21, Table V), the free ferrite content becomes excessive and leads to an unduly low impact value at room temperature (1 ft.-lb.). A 3 to 10 or 12% molybdenum content is provided in the steel.

Cobalt is an essential alloy ingredient to ensure proper microstructural balance in the steel, because cobalt acts as an austenite former at higher temperatures but has only a small effect on the austenite-to-martensite transformation temperature (the Ms temperature). Thus the proper amount of cobalt allows the steel to be hardened and, at the same time, essentially or completely free from delta ferrite. Moreover, cobalt increases the effectiveness of the precipitation of intermetallic compounds in strengthening the steels.

If no nickel is present, a minimum of about 10% cobalt is advantageous for the avoidance of unduly large amounts of delta ferrite in the microstructure (see Steels HW23, 24, and 25, Table V). The test results also show that the tempering resistance as well as the room-temperature and elevated-temperature strengths increase with increasing cobalt content up about 15% (HW25, Table V).

TABLE V.—HARDNESS, TEMPERING RESISTANCE AND MECHANICAL PROPERTIES OF TABLE IV STEELS

| Steel No. | Composition, weight percent |      |      |      |      |     | Free ferrite, percent at— |   |       |    |    |    | Hardness (R <sub>e</sub> ) after tempering 12+2 hr. at— |     |     |     |     |     | Mechanical properties <sup>2</sup> |     |     |     |     |     |           |     |     |     |     |     |     |     |     |     |     |    |    |
|-----------|-----------------------------|------|------|------|------|-----|---------------------------|---|-------|----|----|----|---------------------------------------------------------|-----|-----|-----|-----|-----|------------------------------------|-----|-----|-----|-----|-----|-----------|-----|-----|-----|-----|-----|-----|-----|-----|-----|-----|----|----|
|           | 1,800° F.                   |      |      |      |      |     | 1,900° F.                 |   |       |    |    |    | 1,050° F.                                               |     |     |     |     |     | 1,100° F.                          |     |     |     |     |     | 1,200° F. |     |     |     |     |     |     |     |     |     |     |    |    |
|           | C                           | Cr   | Mo   | W    | Co   | Ni  |                           |   |       |    |    |    |                                                         |     |     |     |     |     |                                    |     |     |     |     |     |           |     |     |     |     |     |     |     |     |     |     |    |    |
| HW12      | 0.04                        | 5.2  | 7.7  | 7.4  | 2.2  | 0   | 0                         | 0 | 39    | 56 | 54 | 49 | 40                                                      | 244 | 288 | 36  | 138 | 165 | 5                                  | 138 | 165 | 20  | 56  | 5   | 138       | 165 | 20  | 56  | 5   | 138 | 165 | 20  | 56  |     |     |    |    |
| HW13      | 0.10                        | 6.2  | 7.4  | 2.2  | 2.1  | 0   | 0                         | 0 | 40    | 63 | 62 | 46 | 46                                                      | 37  | 34  | 223 | 33  | 209 | 29                                 | 42  | 13  | 121 | 145 | 6   | 66        | 6   | 121 | 145 | 20  | 66  | 6   | 121 | 145 | 20  | 66  |    |    |
| HW15      | 0.16                        | 6.3  | 7.6  | 2.1  | 2.1  | 0   | 0                         | 0 | 43    | 62 | 49 | 42 | 36                                                      | 35  | 33  | 223 | 245 | 12  | 40                                 | 7   | 105 | 105 | 134 | 24  | 24        | 105 | 134 | 24  | 24  | 105 | 134 | 24  | 24  | 105 | 134 | 24 | 24 |
| HW14      | 0.05                        | 0.4  | 7.3  | 10.9 | 2.2  | 0   | 0                         | 0 | 36    | 50 | 50 | 44 | 38                                                      | 34  | 30  | 29  | 272 | 11  | 42                                 | 4   | 132 | 158 | 20  | 54  | 20        | 132 | 158 | 20  | 54  | 20  | 132 | 158 | 20  | 54  |     |    |    |
| HW16      | 0.05                        | 2.7  | 7.6  | 10.9 | 2.0  | 0   | 0                         | 0 | 37    | 53 | 52 | 46 | 40                                                      | 38  | 33  | 253 | 290 | 10  | 42                                 | 4   | 142 | 170 | 20  | 53  | 20        | 142 | 170 | 20  | 53  | 20  | 142 | 170 | 20  | 53  |     |    |    |
| HW17      | 0.05                        | 2.8  | 8.3  | 10.9 | 2.3  | 0   | 0                         | 0 | 38    | 55 | 54 | 48 | 40                                                      | 33  | 33  | 244 | 288 | 13  | 42                                 | 4   | 142 | 170 | 20  | 53  | 20        | 142 | 170 | 20  | 53  | 20  | 142 | 170 | 20  | 53  |     |    |    |
| HW12      | 0.04                        | 5.2  | 7.7  | 7.7  | 2.2  | 0   | 0                         | 0 | 39    | 66 | 64 | 49 | 40                                                      | 36  | 33  | 244 | 288 | 13  | 42                                 | 4   | 142 | 170 | 20  | 53  | 20        | 142 | 170 | 20  | 53  | 20  | 142 | 170 | 20  | 53  |     |    |    |
| HW19      | 0.05                        | 11.2 | 7.7  | 11.4 | 2.2  | 0   | 0                         | 0 | 20    | 41 | 66 | 48 | 44                                                      | 44  | 36  | 244 | 288 | 8   | 16                                 | 2   | 116 | 162 | 16  | 45  | 16        | 116 | 162 | 16  | 45  | 16  | 116 | 162 | 16  | 45  |     |    |    |
| HW18      | 0.05                        | 5.8  | 3.0  | 11.0 | 2.1  | 0   | 0                         | 0 | 37    | 56 | 43 | 36 | 25                                                      | 25  | 24  | 176 | 200 | 16  | 58                                 | 12  | 119 | 119 | 24  | 57  | 24        | 119 | 119 | 24  | 57  | 24  | 119 | 119 | 24  | 57  |     |    |    |
| HW12      | 0.04                        | 5.2  | 7.6  | 11.2 | 2.2  | 0   | 0                         | 0 | 39    | 56 | 54 | 49 | 40                                                      | 36  | 36  | 244 | 288 | 13  | 46                                 | 5   | 138 | 165 | 20  | 56  | 20        | 138 | 165 | 20  | 56  | 20  | 138 | 165 | 20  | 56  |     |    |    |
| HW20      | 0.05                        | 5.5  | 10.0 | 11.4 | 2.2  | 0   | 0                         | 0 | 10-15 | 41 | 56 | 55 | 48                                                      | 40  | 40  | 39  | 285 | 10  | 33                                 | 3   | 125 | 164 | 16  | 43  | 16        | 125 | 164 | 16  | 43  | 16  | 125 | 164 | 16  | 43  |     |    |    |
| HW21      | 0.05                        | 5.2  | 15.1 | 11.1 | 2.2  | 0   | 0                         | 0 | 50    | 50 | 46 | 50 | 57                                                      | 52  | 44  | 44  | 244 | 288 | 12                                 | 123 | 173 | 10  | 14  | 10  | 123       | 173 | 10  | 14  | 10  | 123 | 173 | 10  | 14  |     |     |    |    |
| HW22      | 0.04                        | 5.3  | 7.6  | 8.0  | 2.1  | 0   | 0                         | 0 | <5    | 38 | 53 | 51 | 46                                                      | 37  | 32  | 256 | 290 | 12  | 49                                 | 5   | 126 | 151 | 20  | 59  | 20        | 126 | 151 | 20  | 59  | 20  | 126 | 151 | 20  | 59  |     |    |    |
| HW22      | 0.04                        | 5.2  | 7.6  | 8.0  | 2.1  | 0   | 0                         | 0 | 39    | 53 | 50 | 44 | 40                                                      | 36  | 36  | 244 | 288 | 13  | 46                                 | 5   | 126 | 151 | 20  | 59  | 20        | 126 | 151 | 20  | 59  | 20  | 126 | 151 | 20  | 59  |     |    |    |
| HW23      | 0.05                        | 5.4  | 7.6  | 8.1  | 2.2  | 0   | 0                         | 0 | 30    | 40 | 33 | 47 | 44                                                      | 36  | 36  | 244 | 288 | 11  | 48                                 | 3   | 138 | 165 | 20  | 62  | 20        | 138 | 165 | 20  | 62  | 20  | 138 | 165 | 20  | 62  |     |    |    |
| HW24      | 0.05                        | 5.4  | 7.4  | 8.1  | 2.2  | 0   | 0                         | 0 | <2    | 37 | 53 | 48 | 39                                                      | 32  | 32  | 288 | 310 | 13  | 44                                 | 3   | 138 | 165 | 20  | 57  | 20        | 138 | 165 | 20  | 57  | 20  | 138 | 165 | 20  | 57  |     |    |    |
| HW25      | 0.05                        | 5.4  | 7.6  | 11.2 | 2.2  | 0   | 0                         | 0 | 38    | 56 | 50 | 42 | 36                                                      | 270 | 310 | 13  | 44  | 3   | 138                                | 165 | 20  | 59  | 20  | 138 | 165       | 20  | 59  | 20  | 138 | 165 | 20  | 59  |     |     |     |    |    |
| HW27      | 0.07                        | 5.3  | 7.4  | 11.6 | 2.2  | 0   | 0                         | 0 | 40    | 57 | 55 | 51 | 45                                                      | 37  | 37  | 285 | 309 | 9   | 30                                 | 5   | 138 | 165 | 20  | 56  | 20        | 138 | 165 | 20  | 56  | 20  | 138 | 165 | 20  | 56  |     |    |    |
| HW12      | 0.04                        | 5.2  | 7.7  | 11.2 | 2.2  | 0   | 0                         | 0 | 37    | 56 | 54 | 46 | 38                                                      | 33  | 33  | 235 | 275 | 14  | 47                                 | 8   | 117 | 146 | 24  | 62  | 24        | 117 | 146 | 24  | 62  | 24  | 117 | 146 | 24  | 62  |     |    |    |
| HW26      | 0.04                        | 5.5  | 7.6  | 11.2 | 2.2  | 0   | 0                         | 0 | 37    | 53 | 50 | 44 | 39                                                      | 33  | 33  | 235 | 275 | 16  | 47                                 | 10  | 106 | 126 | 23  | 67  | 23        | 106 | 126 | 23  | 67  | 23  | 106 | 126 | 23  | 67  |     |    |    |
| HW27      | 0.04                        | 5.3  | 7.8  | 11.4 | 2.2  | 0   | 0                         | 0 | 45    | 54 | 53 | 48 | 40                                                      | 40  | 40  | 247 | 286 | 8   | 17                                 | 4   | 130 | 162 | 20  | 61  | 20        | 130 | 162 | 20  | 61  | 20  | 130 | 162 | 20  | 61  |     |    |    |
| HW30      | 0.05                        | 6.1  | 11.4 | 14.6 | 11.4 | 1.2 | 0                         | 0 | 45    | 52 | 52 | 48 | 40                                                      | 39  | 39  | 247 | 286 | 6   | 12                                 | 3   | 122 | 155 | 20  | 62  | 20        | 122 | 155 | 20  | 62  | 20  | 122 | 155 | 20  | 62  |     |    |    |

<sup>1</sup> Heat treatment: Austenitized at 1,800° F. for ½ hour, oil quenched, tempered at 1,100° F., 2+2 hour.<sup>2</sup> Heat treatment: Austenitized at 1,800° F. for ½ hour, oil quenched, tempered, at 1,100° F., 2+2 hour.

3,508,912

Increasing cobalt above the 15% level (HW41, Table V) leads to no further significant increase in strength and the room-temperature ductility is lowered. Thus an upper limit of 15% is used for cobalt with a lower limit of 8% being used to provide freedom from delta ferrite.

Nickel can be used to replace cobalt (HW12, 26, and 27, Table V). The inclusion of up to 2% nickel (HW12 vs. 24, Table V) has beneficial effects on virtually all properties investigated. If used in excess nickel is expected to cause the steel to form an austenitic structure at the usual tempering and service temperatures; as a result, the strength is reduced. Hence, up to 4% nickel may be present in the steel.

Tungsten may be used as a partial or complete substitute for molybdenum (Steels HW29 and 30, Table V). The amount of tungsten should be about twice the amount of molybdenum it replaces.

Generally, the steels investigated contained from 0.01

to 0.02% nitrogen; these amounts are regarded as incidental. In accordance with the general theory of alloying

elements of the new steels) may be added in any quantity required to effect the desired carbon stabilization. The exact amount of any one such additive element, or any combination thereof, is readily determinable by well known stoichiometric principles, i.e., the fixed proportion of carbon and carbide-former in the resultant carbide. In general, these purposes are served by addition of such carbide (and nitride) forming elements in amounts up to about 10 times the total carbon plus nitrogen contents of the steels. The carbides, nitrides, or carbonitrides thus produced have the advantage of conferring some additional hardness and wear resistance on the steels. Moreover, the addition of such carbide-forming elements, as, for example, columbium, tantalum, vanadium, titanium, zirconium, and hafnium, affords a means of reducing the level of matrix carbon (and nitrogen), especially in those instances wherein these elements are present on the high sides of their respective or total

range. For the purpose of so stabilizing the steels, amounts of such strong carbide formers (stronger than molybdenum—the strongest carbide former of the purpose of steel) treatment: Austenitized at 1,800° F. for ½ hour, oil quenched, tempered, at 1,100° F., 2+2 hour.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

As to the sulfur and phosphorus contents, no criticality is known. The amounts resulting from good conventional steelmaking practice would be acceptable.

Addition of strong carbide (and nitride and carbonitride) forming elements, such as columbium, tantalum, vanadium, titanium, zirconium, and hafnium, affords a means of reducing the level of matrix carbon (and nitrogen), especially in those instances wherein these elements are present on the high sides of their respective or total range. For the purpose of so stabilizing the steels, amounts of such strong carbide formers (stronger than molybdenum—the strongest carbide former of the purpose of steel) treatment: Austenitized at 1,800° F. for ½ hour, oil quenched, tempered, at 1,100° F., 2+2 hour.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

In general the manganese contents of the steels were less than 0.25%. Manganese up to about 1% is feasible. The experimental steels contained usually less than 0.15% silicon, but any silicon content up to about 0.50% is considered possible if proper steps are taken to counterbalance the fertilizing effect of silicon.

which excessive grain growth is most pronounced. For this purpose, carbon is usefully present on the high side of its contemplated range. This further advantage is illustrated by the results of a further series of tests of steels having compositions as given in the following Table VI:

| Steel No.: | Composition, weight percent |      |       |       |      |      |      |      |          |
|------------|-----------------------------|------|-------|-------|------|------|------|------|----------|
|            | C                           | Cr   | Mo    | Co    | Ni   | Mn   | Si   | Cb   | Fe       |
| HS-11      | 0.06                        | 4.57 | 11.34 | 14.7  | 2.1  | 0.17 | 0.10 |      | Balance. |
| HS-11M     | 0.125                       | 4.51 | 11.71 | 14.69 | 2.22 | 0.65 | 0.16 | 0.19 | Do.      |

The steels of Table VI were austenitized at 2200° F. for 10 minutes, oil quenched, the grain size determined, and the steels were then tempered at 1000° F. (2+2 hours for Steel HS-11M, 2+2+4 hours for Steel HS-11), and tested for impact strength. The results of such tests are given in Table VII:

| Steel No.: | Tempered hardness, R <sub>c</sub> | ASTM grain size |      | Charpy C-notch impact strength, foot-pounds |
|------------|-----------------------------------|-----------------|------|---------------------------------------------|
|            |                                   | No.             | size |                                             |
| HS-11      | 66                                | 2-3             |      | 2                                           |
| HS-11M     | 67                                | 5-6             |      | 4                                           |

It will be seen from Table VII that the columbium-containing steel had a significantly smaller grain size and higher impact strength than the columbium-free steel. Somewhat greater amounts of carbide-formers, consistent with maintenance of a delta ferrite-free structure, may be used to further enhance this desirable effect.

As aforesaid, the steels of the invention are hardened and strengthened by precipitation of intermetallic compounds upon aging. Molybdenum is an important element in this regard, and is believed to combine with iron to form compounds, as an Fe<sub>2</sub>Mo-type Laves phase, and with iron and chromium to form a chi phase. Tungsten is similarly useful, probably forming similar intermetallic compounds, as Fe<sub>2</sub>W, and accordingly, molybdenum in the new steels may in general be substituted, in whole or in part, by tungsten, on a basis of 2 parts by weight of tungsten to one part by weight of substituted molybdenum, due to the greater atomic weight of tungsten.

Graph A of FIG. 4 is illustrative of the effect of molybdenum content upon the maximum attainable hardness upon tempering (at 1050° F.). From that graph, it will be seen that maximum hardness is achieved at a molybdenum content of about 10 to 12%. Hardnesses of 50 to 55 R<sub>c</sub> are readily obtainable when molybdenum is present in amounts of 7 to 8%.

Molybdenum also is productive of temper resistance in the new steels, this property increasing with increasingly larger quantities of that element. Graphs B, C and D of FIG. 4 are illustrative of this effect of molybdenum, wherein the molybdenum content is related to the percentage difference in the maximum attainable tempered hardness (1050° F. temper) and the hardness retained after progressively higher tempering temperatures. This effect is particularly evident at the more rigorous conditions of 1400° F. and 1300° F. illustrated by Graphs B and C, respectively. In both instances, the hardness loss on tempering reduces to a relatively low, constant percentage level in the molybdenum range of 10-15%. The same is true, though the change is less abrupt, at the 1200° F. tempering temperature.

The substitutability of tungsten for molybdenum is illustrated by the Table V data for Steels HW12, 29 and 30. In the latter two steels, tungsten was substituted for molybdenum, in steel HW29 the substitution being on a 48% basis (considering the combined effective amount of these two elements as percent Mo+1/2% W), and in

steel HW30 the substitution being complete. FIG. 5 graphically illustrates the Table V data on the tensile strength properties of these three steels, and it will be seen from that figure that both room temperature and 1100° F. tensile properties, both yield strength andulti-

mate tensile strength, are substantially unaffected by this substitution. However, it will be further noted from the Table V data, that the ductility values of the higher tungsten steels are generally lower than those of the steels having a greater proportion of molybdenum. For this reason, as well as because of the higher cost of tungsten and the larger amounts required to achieve the properties obtainable with smaller amounts of the less expensive molybdenum, the latter element is preferred to tungsten in our steels.

A further experimental steel, Steel No. 64-374 was prepared having the following composition:

Steel 64-374:

|    |    |       |
|----|----|-------|
| 30 | C  | 0.06  |
|    | Cr | 4.57  |
|    | Mo | 11.34 |
|    | Co | 14.69 |
|    | Ni | 2.0   |
| 35 | Mn | 0.70  |
|    | Si | 0.11  |
|    | Fe | Bal.  |

This steel, by reason of proper balance of ferrite- and austenite-formers, contained no free ferrite after austenitizing at 2200° F., although it contained 11.34% molybdenum. Upon quenching and tempering at 1000° F. for 2+2+4 hours, this steel exhibited a hardness of 67 R<sub>c</sub>. Moreover, the steel also exhibited a highly superior resistance of softening, as illustrated by the graphs of FIG. 6, wherein Graph E represents the tempering resistance of Steel 64-374, and Graph F that of a commonly used high speed steel, AISI Type M-2, containing 0.85% C, 0.30% Mn, 0.30% Si, 4.15% Cr, 1.95% V, 6.40% W, 5.0% Mo, balance essentially Fe. The tempering parameter used in FIG. 4 is the common Larsen-Miller parameter

$$P = T(20 + \log t) \times 10^{-3}$$

wherein:

T=temperature, ° R, and

t=time, hours.

It will be seen from these two graphs that Steel 64-374, at practically all parameter values, is equivalent or superior, in tempering resistance, to the M-2 steel, and at parameters above about 34, representing more rigorous conditions of time and temperature, the experimental steel is markedly superior in this regard to the prior art high speed steel.

Steel No. 64-374 was further compared with respect to cutting tool life, to commercial high speed tool steel of the general AISI Type M-2 composition (0.85% C, 0.30% Mn, 0.30% Si, 4.15% Cr, 1.95% V, 6.40% W, 5.00% Mo, balance Fe), and with the same composition having a higher (0.96%) carbon content. The workpiece was commercial AISI H-13 hot work steel (0.40% C, 0.40% Mn, 1.10% Si, 5.00% Cr, 1.10% V, 1.35% Mo, balance Fe) hardened to 28-30 R<sub>c</sub>. The cutting tools were approximately 1/2-inch square by 1 1/2 inches in length. Cutting was done dry, the depth of cut was 0.062 inch and feed was 0.010 inch per revolution. The tool geometry was 3°, 6°, 10°, 10°, 10°, 10° and the nose radius was

0.030 inch. The results of such tests are set out in the following Table VIII.

TABLE VIII

| Steel designation: | Average tool hardness, R <sub>e</sub> | Average tool life, minutes plus turning |               |
|--------------------|---------------------------------------|-----------------------------------------|---------------|
|                    |                                       | 60 s.f.p.m.                             | 65 s.f.p.m.   |
| (.85C)M2           | 65.5                                  | 1 23.4(1)                               | 2 14.3±2.1(2) |
| (.96C)M2           | 66.5                                  | 1 38.1(1)                               | 2 25.1±1.0(3) |
| Alloy 64-374       | 65.5/66.0                             | 2 40.0±2.0(2)                           | 2 29.6±3.9(6) |

<sup>1</sup> Figure in parentheses is the number of test cuts.

<sup>2</sup> Second figure is the standard deviation ( ) of the tests conducted.

ound precipitation (also facilitated, as noted, by the cobalt addition). For this purpose, a large spread between quenched (or quenched and refrigerated) hardness and maximum attainable tempered hardness is desirable. FIG. 8 illustrates the effect of cobalt on this property. Thus, the three graphs, G, H and I, there appearing relate the percentage of cobalt in the four steels HW23, 24, 25 and 41, with the difference (Rockwell C points) between the untempered hardness and the tempered hardness at, respectively, 1050° F., 1100° F. and 1200° F. Maximum hardness spread is seen from these graphs to occur, in each instance, at cobalt values of about 14 to 15.5%.

TABLE IX

| Steel: | Percent cobalt | Percent nickel | Total percent Co+Ni | Hardness, R <sub>e</sub> , at indicated tempering temperatures |           |           |           |           | Hardness loss, ° F., percent |
|--------|----------------|----------------|---------------------|----------------------------------------------------------------|-----------|-----------|-----------|-----------|------------------------------|
|        |                |                |                     | 1,050° F.                                                      | 1,100° F. | 1,200° F. | 1,300° F. | 1,400° F. |                              |
| HW27   | 6.8            | 6.6            | 13.4                | 53                                                             | 50        | 44        | 39        | 39        | 24.5                         |
| HW26   | 9.2            | 4.0            | 13.2                | 54                                                             | 52        | 46        | 38        | 38        | 29.7                         |
| HW12   | 11.2           | 2.2            | 13.4                | 56                                                             | 54        | 49        | 40        | 36        | 35.6                         |
| HW25   | 14.2           | —              | 14.2                | 58                                                             | 55        | 50        | 42        | 35        | 37.3                         |

It will be seen from the Table VIII data that, under the stated test conditions, the age-hardened steel No. 64-374 tools cut about twice as long as the 0.85% carbon M-2 high speed steel tools, and about equally as long as did the 0.96% M-2 tools.

The effect of cobalt upon tensile properties is graphically illustrated by FIG. 7, erected upon the data of Table V. From FIG. 7, it will be seen that maximum room temperature yield and ultimate tensile strengths are obtained by the inclusion in the contemplated steels of about 15% to 16% cobalt. Similarly, maximum values of these

In addition to the foregoing advantages, the steels of the invention also exhibit excellent resistance to heat checking which, as above-mentioned, is an important property of hot work tool steels. Thus, a representative steel 30 of the invention, of a composition approximately that of Steel No. HW12 of Table IV, was compared, for heat check resistance, to a nominal AISI H-13 type steel—a commonly used prior art hot work steel. A specially melted low residual Type H-12 was also used in these 35 comparison tests, the actual steel compositions being as given in Table X below.

TABLE X

| Steel:               | Bar No. | Composition, weight percent |      |       |       |      |      |      |      |      |       |
|----------------------|---------|-----------------------------|------|-------|-------|------|------|------|------|------|-------|
|                      |         | C                           | Mn   | P     | S     | Si   | Cr   | Mo   | V    | Ni   |       |
| HW12                 | 241     | 0.058                       | 0.06 | —     | —     | —    | 0.08 | 4.64 | 7.52 | 1.93 | 11.30 |
| H-13                 | 63-496  | 0.39                        | 0.37 | 0.016 | 0.016 | 1.11 | 5.06 | 1.38 | 1.07 | 0.20 | Do.   |
| H-13 (low residual). | 65-171  | 0.39                        | 0.07 | 0.006 | 0.016 | 0.18 | 4.93 | 1.35 | 1.17 | —    | Do.   |

properties at elevated temperatures, e.g., 1100° F., are obtained at about the 15% cobalt level. Usefully high strength properties, at both room temperature and 1100° F., are obtained at cobalt levels of 10 or 11% upwardly to the aforesaid maximum value.

The aforementioned test set also shows the appearance, in the tested nominally 0.05% C-5.4% Cr-7.5% Mo base composition, of a substantial proportion (30-40 volume percent) of delta ferrite at the 8% cobalt level. Traces of this phase still remained at the 11% cobalt level.

As previously mentioned, the steels of the invention, in large part due to the aforementioned part played by the cobalt addition, are machinable in the austenitized condition and thereafter hardenable by intermetallic com-

50 The heat check test consisted of a 4-second immersion of the test specimens (mounted on a rod-like spindle) into a molten lead bath at a temperature of 1225 to 1250° F., followed by a 1.5 second quench in a 170 to 190° F. water bath, after which the specimens were dried above the lead bath for 5 seconds. This test cycle was repeated at a rate of about 3 cycles per minute.

Each test specimen was in the form of a circular body having a centrally apertured hub and circumferential flange extending from the midline of the hub. The flange had an outside diameter of 2.000 inches and a thickness of 0.075 inch, while the hub had an outside diameter of 1.500 inches, a thickness of 0.350 inch and a hub aperture of  $3\frac{3}{4}$  inch.

Prior to testing, the specimens were heat treated as shown in Table XI.

TABLE XI

| Test sample: | Austenitization |            |                   |
|--------------|-----------------|------------|-------------------|
|              | Temp., ° F.     | Time, hrs. | Cooling treatment |
| 241-A, B     | 1,800           | 0.5        | Oil quench        |
| 63-496-4, 5  | 1,850           | 0.5        | Air cool          |
| 65-171-1, 2  | 1,850           | 0.5        | do                |

The results of the heat check tests are given in Table XII.

conditions due to the high temperature differentials so produced.

TABLE XII

| Steel                         | Specimen No. | Position <sup>1</sup> | Hardness, R <sub>o</sub> | Heat check index, HC at indicated number of heat check cycles |                |                 |               |    |    |               |    |     |               |     |                |                |                |                |
|-------------------------------|--------------|-----------------------|--------------------------|---------------------------------------------------------------|----------------|-----------------|---------------|----|----|---------------|----|-----|---------------|-----|----------------|----------------|----------------|----------------|
|                               |              |                       |                          | 10,000 cycles                                                 |                |                 | 12,500 cycles |    |    | 15,000 cycles |    |     | 17,500 cycles |     |                | 25,000 cycles  |                |                |
|                               |              |                       |                          | N <sup>2</sup>                                                | L <sup>3</sup> | HC <sup>4</sup> | N             | L  | HC | N             | L  | HC  | N             | L   | HC             | N              | L              | HC             |
| HW12-----                     | 241-A        | 3                     | 52.3                     | 0                                                             | 0              | 0               | 0             | 0  | 0  | 0             | 0  | 0   | 0             | 0   | 0              | 0              | 0              | 0              |
| HW12-----                     | 241-B        | 7                     | 53.0                     | 0                                                             | 0              | 0               | 0             | 0  | 0  | 0             | 0  | 0   | 0             | 0   | 0              | 0              | 0              | 0              |
| AISI H-13-----                | 63-496-4     | 2                     | 44.4                     | 1                                                             | 6              | 6               | 5             | 28 | 63 | 13            | 56 | 202 | 18            | 84  | 356            | <sup>5</sup> F | <sup>5</sup> F | <sup>5</sup> F |
| AISI H-13-----                | 63-496-5     | 6                     | 44.2                     | 2                                                             | 5              | 7               | 5             | 30 | 67 | 13            | 53 | 191 | 16            | 68  | 283            | <sup>5</sup> F | <sup>5</sup> F | <sup>5</sup> F |
| AISI-H-13 (low residual)----- | { 65-171-1   | 4                     | 46.3                     | 0                                                             | 0              | 0               | 2             | 16 | 23 | 5             | 40 | 89  | 11            | 88  | 292            | <sup>5</sup> F | <sup>5</sup> F | <sup>5</sup> F |
|                               | 65-171-2     | 9                     | 46.9                     | 0                                                             | 0              | 0               | 0             | 0  | 3  | 22            | 38 | 7   | 56            | 148 | <sup>5</sup> F | <sup>5</sup> F | <sup>5</sup> F |                |

<sup>1</sup> Indicated number is position of test specimen (a total of 9 specimens were used) on the holding spindle, from left to right as viewed from the front of the test apparatus.

<sup>2</sup> N=total number of cracks in specimen flange.

<sup>3</sup> L=sum of the lengths of all cracks in specimen flange.

<sup>4</sup> HC=Heat Check Index=I/N.

<sup>5</sup> Specimen Nos. 63-496-4, 5 were inserted after 1,000 cycles had been accumulated on other Table IX specimens.

<sup>6</sup> F, indicates specimen heat checking so extensive as to be considered to have completely failed beyond usefulness in any conceivable die casting end use, prior to indicated number of cycles.

From the results of Table XII, it is seen that heat checking of AISI Type H-13 (Specimen Nos. 63-496-4, 5) hot work steel as initiated at about 10,000 cycles, whereas, in the case of the low-residual H-13 steel, heat checking commenced between 12,500 and 15,000 cycles. After 17,500 cycles, both prior art steels had exhibited complete failure. On the other hand, the inventive steel HW-12 had not even started to show heat check cracks at 25,000 cycles when the test was discontinued.

It was further observed that the flange surfaces of the conventional and the modified (low-residual) prior art steels had eroded considerably, by scaling and decarburization, during the test, whereas the inventive steel was essentially uneroded and was readily cleaned to present the original smooth surface appearance.

Such properties confer on the new steels a high degree of utility in application to elevated temperature end uses, as in the forging of high temperature materials, in the extrusion of brass, in the construction of spreaders and cores in aluminum castings—where the metal is subjected to the full impact of an injected stream of aluminum, in the construction of turbine buckets, blades, etc. Indeed, the new steels are useful in most hot work applications wherein very high surface temperatures, e.g. 1200-1700° F. are encountered. Water cooling can be used in such applications with relative immunity from the cracking usually exhibited by prior art hot work steels under such

20 What is claimed is:

1. A hot work steel consisting essentially, by weight percent, of about

25 Carbon + nitrogen ----- Up to 0.08.

Chromium ----- 2.5 to 6.

Molybdenum ----- 3 to 12.

Cobalt ----- 8 to 15.

Nickel ----- Up to 4.

Cobalt + nickel ----- 10 to 18.

Manganese ----- Up to 1.

30 Iron ----- Balance, except for incidental steelmaking impurities.

35 2. The steel of claim 1 wherein up to 100% of the molybdenum content is replaced by tungsten on a 2 to 1 weight basis.

#### References Cited

#### UNITED STATES PATENTS

|           |         |                        |
|-----------|---------|------------------------|
| 2,099,509 | 11/1937 | Blessing.              |
| 2,504,453 | 4/1950  | Rotherham.             |
| 2,598,714 | 6/1952  | Nelson.                |
| 3,154,412 | 10/1964 | Kasak ----- 75—128.9   |
| 3,231,709 | 1/1966  | Folay ----- 75—128.9   |
| 3,251,683 | 5/1966  | Hammond ----- 75—128.9 |

45 HYLAND BIZOT, Primary Examiner

U.S. CL. X.R.

75—126

UNITED STATES PATENT OFFICE  
CERTIFICATE OF CORRECTION

Patent No. 3,508,912 Dated April 28, 1970

Inventor(s) Vijay K. Chandhok and August Kasak

It is certified that error appears in the above-identified patent and that said Letters Patent are hereby corrected as shown below:

Column 4, line 10, after "impart", delete --to--;

Table II, column 3, under "C" line 2, change "0.006" to --0.096--; same Table, column 4, under "Cr" last line, change "3.59" to --5.39--;

Table III, column 1, under "Steel", line 1, change "HW1, 0.10C-6Cr-10Mo-14Co" to --HW1, 0.10C-5Cr-10Mo-14Co--;

Table V, column 12, line 17 under 1,100°F, change "59" to --55--; same Table, column 13, line 19 under 1,200°F, change "40" to --49--; same Table, column 15, line 5 under 1,400°F, change "40" to --30--;

Column 10, middle paragraph, last line, change "purpose" to --purposeful--;

Column 12, line 43, change "of" (first occurrence) to --to--;

Column 14, line 34, change "H-12" to --H-13--;

Column 14, line 61, after "hub" delete --hand--.

SIGNED AND  
SEALED

SEAL)

Attest:

Edward M. Fletcher, Jr.

Attesting Officer

SEP 29 1970

WILLIAM E. SCHUYLER, JR.  
Commissioner of Patents